

Oct. 28, 1930.

J. W. LITTLEFORD

1,780,022

FLOTATION CONCENTRATION OF PHOSPHATIC MATERIAL

Filed July 3, 1928



INVENTOR

John W. Littleford

BY

Williams, Rich & Morse

ATTORNEYS

## UNITED STATES PATENT OFFICE

JOHN W. LITTLEFORD, OF ALAMEDA, CALIFORNIA, ASSIGNOR TO MINERALS SEPARATION NORTH AMERICAN CORPORATION, OF NEW YORK, N. Y., A CORPORATION OF MARYLAND

## FLOTATION CONCENTRATION OF PHOSPHATIC MATERIAL

Application filed July 3, 1928. Serial No. 290,284.

This invention relates to the concentration by flotation of phosphatic material and is herein illustrated as carried out in such apparatus as is often used for the froth-flo-  
5 tation concentration of ores, although under the present procedures often no froth is formed of the usual type. The process is herein illustrated as applied to the so-called phosphate rock of Florida and to the tailings  
10 residue or débris from sieving processes of concentrating that material. The same pro-  
cedures have been found useful with Tennessee phosphate rock.

It is known that the amount of the agents  
15 needed to effect the flotation of the phosphatic concentrate may be greatly reduced by elimination of the phosphatic and some other slimes from the ground or fine mate-  
rial.

It has now been found that the amount of  
20 the agents needed may be further diminished by so conducting the aerating agitation as to avoid as much as possible agitation in ex-  
cess of that necessary to raise the float con-  
centrate. It has also now been found that  
25 the order of adding certain of the agents may be important in permitting the mini-  
mum amount of agent or agents to be effec-  
tive. Under large-scale conditions, where  
30 the price of the available agents is of vital  
importance, best results with minimum con-  
sumption of agents have been obtained in  
the examples hereinafter given by adding  
35 caustic soda solution to a thick pulp in a  
screw conveyor serving as a preliminary  
mixer, and thereafter, during the mixing,  
adding soap or a soap-forming material,  
such for example, as oleic acid, and also add-  
40 ing, with the oleic acid or before or after  
adding the oleic acid, an agent commonly  
called a collector, such as fuel oil.

The process has been found to work satis-  
factorily in an apparatus such as is dia-  
grammatically shown in the accompanying draw-  
45 ing, in which a pulp carrying about 60% to  
70% deslimed solids, finer than 14-mesh,  
flows down a launder 1 into a screw conveyor  
2 of an ordinary type having a trough 3, in  
which lies a revolving screw 4 so that the  
50 pulp flows along to a rotary pump 5, at the

lower end of a conduit 6, by which pump  
the pulp is forced up through the conduit 6.  
As the thick pulp flows along the mixer 2  
it receives, first, a small amount of caustic  
soda in solution through a drip dia-  
grammatically shown at 7. Later, after the cau-  
55 stic soda is thoroughly distributed, the pulp  
receives through a drip or drips, dia-  
grammatically shown at 8, red oil (oleic acid) and  
fuel oil, although the fuel oil may be added  
before or after the red oil. Later, after the  
60 oils have been thoroughly distributed, there  
is added water from a tap dia-grammatically  
shown at 9 to make a 4 to 1 thinned pulp.

The pump 5 delivers the thinned pulp  
through the conduit 6 to the head of a cas-  
cade froth-flo-  
70 tation cell 10 having a tank  
body 11, a pipe 12 through which the pulp  
falls on to a deflector 13 such as is shown  
in United States patent to Court No. 1,470,  
350, of October 9, 1923. The Cascade flo-  
tation machine shown has three cells. As the  
pulp falls in the pipe 12 it gathers air which  
enters through  $\frac{3}{8}$  inch openings 14 near the  
top of the pipe 12. The aerated pulp is de-  
flected upwardly by the deflector 13 through  
an egg-crate baffle 15 above the deflector, and  
the float overflows past a lip 16 around the  
75 tank 11. A tailings discharge valve 17 is  
provided in the center of the bottom of the  
tank 11 provided with a control handle 18,  
but there is also a weir-overflow tailings dis-  
charge 26 to determine the pulp level in rela-  
tion to the overflow lip 16. The weir, in the  
80 form illustrated, is in the wall of a small  
separate compartment having a feed open-  
ing 27 admitting pulp from below the de-  
flector 13 of the tank body 11 and open to  
the weir 26 over which the pulp flows into  
85 a tailings launder 28. The latter delivers the  
weir-overflow to a tailings discharge pipe 29  
provided with air-admitting openings 8.

The overflowing float in the launder 19  
around the lip 16 runs down a launder 20 to  
a four cell subaeration froth-flo-  
90 tation machine 31 of the general type shown in the  
patent to Wilkinson and this applicant, No.  
1,588,077, dated June 8th, 1926, where the  
float is cleaned by further flotation. As the  
float passes down the launder 20 it is joined  
100

by similar overflowing float from the second cascade concentration cell 22 which treats the tailings from the first cell 11, and is also joined by the overflowing float from a third cell 23 which in turn treats the tailings from the second cell 22, all these three cells being substantially identical. Make up water may be added in the pipe 12 by a valved supply 32.

It is found that a much cleaner float is obtained if the cells include a doubly sloped baffle 24 around the sides below the overflow lip, forming a constriction so that the float rises near the center of the cell and flows over a quiet zone above the baffle 24 because that baffle keeps rising material away from the lip. It is also found advantageous to enclose the central third, or so, of the cells 11, 22 and 23 with baffles 30 which prevent surgings of the pulp from reaching their overflow lips 16.

The cells of the four-cell subaeration machine 21 are found to deliver a cleaner float if provided with paddles 31 for assisting the prompt overflow of the float concentrate. The tailings from the machine 21 form a middling which is returned to the pump 5.

In the devices just described the thick pulp of deslimed crude phosphatic material is gently but thoroughly mixed, first with the caustic alkali, then with the red oil and fuel oil, and the pulp is then thinned and concentrated by flotation with a minimum of agitation. By this procedure the usually muddy mill water absorbs a minimum quantity of the added agents, yet the phosphatic material is adequately treated with the agents.

It does not appear to be necessary that the caustic soda remain in the pulp water. Useful results were obtained when the pulp water was drained off after adding the caustic soda, the solids cautiously washed, and then made into a pulp with water and floated with the aid of oleic acid. It has also been found possible to obtain useful results by adding a less amount of caustic soda as a first addition to the thick pulp, following this with the addition of an oleic acid soap instead of red oil.

It has been found that the cost of agents consumed in the foregoing procedures is about one fourth of the cost of the agents consumed in procedures hitherto used.

*Example 1.*—In one laboratory test run tailings from a concentration operation effected by screening Mulberry, Florida, rock, finer than 20-mesh and deslimed, were gently stirred by hand as a thick pulp containing 70% solids with 0.5 pounds of caustic soda added in solution. Then there was added 0.72 pounds per ton of oleic acid during the continuance of the stirring, followed by 4.0 pounds of fuel oil, all per ton of dry material. The resulting pulp was then thinned to about 4 to 1 with mine water, containing the usual slimes, and agitated in a laboratory froth-flotation spitzkasten sub-aeration ma-

chine and the float removed for three minutes. The results are shown in the following table in which B. P. L. represents bone phosphate of lime:

|            | Wts.     | B. P. L. | Recoveries | 70 |
|------------|----------|----------|------------|----|
|            | Per cent | Per cent | Per cent   |    |
| Heads..... | 100      | 33.67    | 100        |    |
| Conc.....  | 42.4     | 72.98    | 91.8       |    |
| Tails..... | 57.6     | 4.82     | 8.2        | 75 |

*Example 2.*—In another test clear Long Island City, N. Y., tap water was used in the same procedure, except that the added agents were used in less quantity, viz, 0.4 pounds of caustic soda, 0.56 pounds of oleic acid, and 1.68 pounds of fuel oil all per ton of solids. The first concentrate was cleaned, yielding a finished concentrate and a middling. The results are shown in the following table:

|            | Wt.      | B. P. L. | Recoveries | 80 |
|------------|----------|----------|------------|----|
|            | Per cent | Per cent | Per cent   |    |
| Heads..... | 100      | 32.2     | 100        |    |
| Conc.....  | 40.6     | 71.2     | 89.7       |    |
| Midd.....  | 8.9      | 14.4     | 4.0        |    |
| Tails..... | 50.5     | 4.0      | 6.3        |    |

The foregoing test shows a further reduced consumption of agents.

*Example 3.*—On a large scale test run in which about 20 tons of concentrates were obtained in seven hours, treating tailings of the same character, but only partly deslimed, the apparatus shown in the drawing was used in the manner above described. The caustic solution was added at the rate of 0.3 pounds of the dry caustic per ton of solids. There was also added 0.7 pounds of oleic acid and 3.0 pounds of fuel oil, both per ton of solids. There was also added at the subaeration cells 21 of the accompanying drawing, 0.15 pounds of steam-distilled pine oil per ton of solids in the original feed. The results are shown in the following table, the higher bone phosphate of lime content of tailing being due to the deleterious action of the slimes present:

|            | B. P. L. | Recoveries | 100 |
|------------|----------|------------|-----|
|            | Per cent | Per cent   |     |
| Heads..... | 29.78    | 100        |     |
| Conc.....  | 71.89    | 64.1       |     |
| Tails..... | 14.48    | 35.9       |     |

Rapid overflow of the float both in the cascade machine and in the sub-aeration machine improved the grade of the float concentrate, and increased the recovery.

Other agents than the foregoing have proved useful, but seem to add nothing commercially profitable. Water gas tar which also contains a large proportion of insoluble oily material is about as effective as fuel oil. Carbonate of soda is not quite as effective as

caustic soda and the addition of pine oil causes more bubbles to form and on occasions has improved the results, as in the third example.

5 *Example 4.*—In one test of the same material, using the mine water at Mulberry, the procedure of the first of the foregoing tests was used, save that 0.8 pounds of caustic soda, 0.9 pounds of oleic acid, and 6.0 pounds of 10 fuel oil were used per ton of solids, and there was further added in the flotation machine 0.15 pounds per ton of steam distilled pine oil. The results are shown in the following table:

| 15         | Wt.      | B. P. L. | Recoveries |
|------------|----------|----------|------------|
|            | Per cent | Per cent | Per cent   |
| Heads..... | 100      | 34.77    | 100        |
| Concs..... | 43.5     | 73.5     | 93.2       |
| Tails..... | 56.5     | 4.3      | 6.8        |

20 *Example 5.*—A parallel test in the absence of pine oil yielded the following results:

| 25         | Wt.      | B. P. L. | Recoveries |
|------------|----------|----------|------------|
|            | Per cent | Per cent | Per cent   |
| Heads..... | 100      | 32.60    | 100        |
| Concs..... | 39.2     | 73.48    | 88.4       |
| Tails..... | 60.8     | 7.57     | 11.6       |

30 In other tests a soap solution was added instead of oleic acid.

35 *Example 6.*—In one such test phosphatic material of the same kind was made into a thick pulp with Long Island City tap water, and to this was added 0.2 pounds of caustic soda per ton, and then 1.4 pounds of soap per ton, containing 1.2 pounds oleic acid per ton. There was also added 1.68 pounds per ton of 40 fuel oil. The pulp was then thinned to about a 4 to 1 pulp with the same water and a float concentrate obtained in the testing machine and then recleaned in the same machine to yield a finished concentrate and a middling.

45 The results are shown in the following table:

| 50         | Wt.      | B. P. L. | Recoveries |
|------------|----------|----------|------------|
|            | Per cent | Per cent | Per cent   |
| Heads..... | 100      | 31.4     | 100        |
| Concs..... | 35.8     | 75.8     | 86.5       |
| Midd.....  | 8.4      | 22.0     | 5.9        |
| Tails..... | 55.8     | 4.3      | 7.6        |

55 *Example 7.*—Results seem to be little affected by the method of adding the fuel oil. In one test the same procedures were used except that 0.6 pounds of caustic soda were used and 0.8 pounds of oleic acid were used in a 60 mixture with 6 pounds of fuel oil, all per ton of solids. The pulp was then thinned to about a 4 to 1 pulp with the same water and a float concentrate obtained in the testing machine and then recleaned in the same machine to yield a finished concentrate and a middling.

The results are shown in the following table:

|            | Wt.      | B. P. L. | Recoveries |
|------------|----------|----------|------------|
|            | Per cent | Per cent | Per cent   |
| Heads..... | 100      | 35       | 100        |
| Concs..... | 42.8     | 71.88    | 88         |
| Midd.....  | 7.4      | 13       | 2.7        |
| Tails..... | 49.8     | 6.5      | 9.3        |

Having thus described certain embodiments of my invention what I claim is:

1. The process of concentrating phosphate-bearing material which consists in mixing a pulp of the material relatively free from slimes with alkali, thereafter mixing it with a float-assisting substance, agitating to produce a float concentrate, and separating the float.

2. The process of concentrating phosphate-bearing material which consists in mixing a thick pulp of the material relatively free from slimes with caustic soda, thereafter mixing it with a float-assisting substance, thinning the pulp, agitating the thinned pulp to produce a float concentrate, and separating the float.

3. The process of concentrating phosphate-bearing material which consists in mixing a thick pulp of the material relatively free from slimes with caustic soda, thereafter mixing it with a float-assisting substance, thinning the pulp, subjecting the thinned pulp to a cascade flotation operation to produce a float concentrate, and separating the float.

4. The process of concentrating phosphate-bearing material which consists in mixing a pulp of the material relatively free from slimes with alkali, thereafter mixing it with a soap-forming substance, agitating to produce a float concentrate, and separating the float.

5. The process of concentrating phosphate-bearing material which consists in mixing a thick pulp of the material relatively free from slimes with caustic soda, thereafter mixing it with a soap forming substance, thinning the pulp, agitating the thinned pulp to produce a float concentrate, and separating the float.

6. The process of concentrating phosphate-bearing material which consists in mixing a thick pulp of the material relatively free from slimes with caustic soda, thereafter mixing it with a soap-forming substance, thinning the pulp, subjecting the thinned pulp to a cascade flotation operation to produce a float concentrate, and separating the float.

7. The process of concentrating phosphate-bearing material which consists in mixing a pulp of the material relatively free from slimes with alkali, thereafter mixing it with a float-assisting material containing a soap-

forming substance, agitating to produce a float concentrate, and separating the float.

8. The process of concentrating phosphate-bearing material which consists in mixing a thick pulp of the material relatively free from slimes with caustic soda, thereafter mixing it with a float-assisting material containing a soap-forming substance, thinning the pulp, agitating the thinned pulp to produce a float concentrate, and separating the float.

9. The process of concentrating phosphate-bearing material which consists in mixing a thick pulp of the material relatively free from slimes with caustic soda, thereafter mixing it with a float-assisting material containing a soap-forming substance, thinning the pulp, subjecting to a cascade flotation operation to produce a float concentrate and separating the float.

10. The process of concentrating phosphate-bearing material which consists in mixing a pulp of the material relatively free from slimes with alkali, thereafter mixing it with oleic acid, agitating to produce a float concentrate, and separating the float.

11. The process of concentrating phosphate-bearing material which consists in mixing a thick pulp of the material relatively free from slimes with caustic soda, thereafter mixing it with oleic acid, thinning the pulp, agitating the thinned pulp to produce a float concentrate, and separating the float.

12. The process of concentrating phosphate-bearing material which consists in mixing a thick pulp of the material relatively free from slimes with caustic soda, thereafter mixing it with oleic acid, thinning the pulp, subjecting the thinned pulp to a cascade flotation operation to produce a float concentrate and separating the float.

13. The process of concentrating phosphate-bearing material which consists in mixing a pulp of the material relatively free from slimes with alkali, thereafter mixing it with oleic acid and an unsaponifiable oil, agitating to produce a float concentrate, and separating the float.

14. The process of concentrating phosphate-bearing material which consists in mixing a thick pulp of the material relatively free from slime with caustic soda, thereafter mixing it with oleic acid and an unsaponifiable oil, thinning the pulp, agitating the thinned pulp to produce a float concentrate, and separating the float.

15. The process of concentrating phosphate-bearing material which consists in mixing a thick pulp of the material relatively free from slimes with caustic soda, thereafter mixing it with oleic acid and an unsaponifiable oil, thinning the pulp, subjecting the thinned pulp to a cascade flotation operation to produce a float concentrate, and separating the float.

16. The process of concentrating phos-

phate-bearing material which consists in mixing a pulp of the material relatively free from slimes with alkali, thereafter mixing with a float-assisting substance, agitating so as to produce a float concentrate in the substantial absence of excess agitation, and rapidly overflowing the float.

17. The process of concentrating phosphate-bearing material which consists in mixing a thick pulp of the material relatively free from slimes with caustic soda, thereafter mixing it with float-assisting substance, thinning the pulp, agitating the thinned pulp in the substantial absence of excess agitation to produce a float concentrate, and rapidly overflowing the float.

In testimony whereof, I have affixed my signature to this specification.

JOHN W. LITTLEFORD.

85

90

95

100

105

110

115

120

125

130